

No. 826,099.

PATENTED JULY 17, 1906.

J. A. GILMAN.

METHOD OF TREATING COPPER AND NICKEL MATTE.

APPLICATION FILED OCT. 21, 1903.



Witnesses:

P. H. Prigetti.  
L. C. Kennedy.Inventor:  
J. A. Gilman.  
By Wright, Brown & Loring  
Attorneys.

# UNITED STATES PATENT OFFICE.

JOHN A. GILMAN, OF WEST FAIRLEE, VERMONT.

## METHOD OF TREATING COPPER AND NICKEL MATTE.

No. 826,099.

Specification of Letters Patent.

Patented July 17, 1906.

Application filed October 21, 1903. Serial No. 177,866.

*To all whom it may concern:*

Be it known that I, JOHN A. GILMAN, of West Fairlee, in the county of Orange and State of Vermont, have invented certain new and useful Improvements in Methods of Treating Copper and Nickel Mattes, of which the following is a specification.

This invention is an improvement on the process described in an application, Serial No. 160,840, of myself and George C. Everett for treating copper and nickel mattes, whereby the matte while in a molten state is finely subdivided into particles by impingement against a mechanical surface, such as that of a screen suitably cooled, the stream of particles being then subjected to the action of the oxygen of the air so as to remove the sulfur from the particles.

The present invention involves the same general principle of operation as in the said application, but whereas according to that application the particles are allowed to descend by gravity until substantially solid and in their descent come into contact with the air which oxidizes the sulfur according to my present improvement the stream of particles is subjected to a lateral current of air produced by a suitable blast or otherwise and is thereby deflected, the object and result being to decrease the height or distance from which the particles must be projected and allowed to fall.

The accompanying drawing represents a sectional view of an apparatus for carrying the process of my said invention into effect, and in said drawing 10 is a vertical tubular stack having a lower horizontal extension 11, which opens into a large closed bin or chamber 12, said extension having an air-inlet 13, 40 into which is inserted a steam-pipe 140 for producing an induced blast of air.

Any other equivalent, such as a fan, may be substituted for the steam-blast.

130 is an outlet or chimney for the gases and excess air, opening to the atmosphere at a suitable height and communicating at its lower end through an aperture 20 with the chamber 12.

Into the stack 10 projects a revolving screen 14, cooled and moistened by a sprinkler 15 for finely subdividing the stream of molten matte into particles, the stream being poured into a spout 16 from a ladle 17 and impinging against a vertical abutment 18, which partially shatters the stream and guides it properly onto the screen. This is

the same means as described in the aforesaid application for subdividing the matte; but it will be understood that any other suitable means may be substituted for performing the aforesaid function or any other function of the apparatus herein described.

In the operation of the invention the stream of particles 19 of molten matte descends by gravity in the stack 10 until it encounters the lateral air blast or current produced in the extension 11, whereupon the particles are deflected laterally and fall onto the floor of the chamber or bin 12, from whence they may be removed as desired. The air-blast has the effect of oxidizing and removing the most of the sulfur from the particles of matte and of shortening the vertical fall of the particles over what would be required without the blast. The particles may, if desired, receive some oxidation in the body of the stack 10, the latter having an opening at its upper end controlled by a lid or valve 21.

By subjecting the matte to an air-current after it has been broken up into particles by mechanical means the particles are very quickly and effectively oxidized and a small pressure only of air is required. The invention also enables me to control the period during which the escape of sulfur takes place. The sulfur will not leave the matte freely until the latter has decreased in temperature to a certain point, and by producing the air-blast at this point I may secure the most effective action of the air. The temperature of the blast may, if desired, be maintained during this period by suitable means, as by means of the steam intermixed therewith or by other suitable device.

I claim—

1. A process for treating copper and nickel mattes which consists in projecting a stream of molten particles of the matte into space and changing its direction by a current of air.

2. A process for treating copper and nickel mattes which consists in finely subdividing the matte while in a molten state, projecting the particles in a stream downwardly by gravity, and blowing the stream laterally with a current of air to remove the sulfur of the particles.

3. A process for treating copper and nickel mattes which consists in finely subdividing the matte while in a molten state by impingement thereof against a mechanical surface, and then subjecting the particles to the

action of oxygen to remove sulfur from the matte.

4. A process for treating copper or nickel sulfid mattes which consists in finely dividing the matte while in a molten state, cooling the particles to a temperature at which the sulfur will freely leave them, and subjecting them to the action of an oxidizing agent, whereby the amount of sulfur in the particles is reduced.

5. A process for treating copper and nickel sulfid mattes which consists in shooting the matte while in a molten state, dropping it through the air by gravity a sufficient distance to cool the particles to a temperature at which the sulfur will leave the matte freely, and blowing the particles laterally

with a stream of air to remove the sulfur of the particles.

6. A process for treating copper or nickel sulfid mattes which consists in finely dividing the matte while in a molten state, dropping the particles by gravity a sufficient distance to reduce their temperature to a degree at which the sulfur will freely leave them, and subjecting them to the action of an oxidizing agent, whereby the amount of sulfur in the particles is reduced.

In testimony whereof I have affixed my signature in presence of two witnesses.

JOHN A. GILMAN.

Witnesses:

R. M. PIERSON,  
A. C. RATIGAN.